

## 1

3,511,663

SILVER HALIDE EMULSIONS CONTAINING 2-AMINO IMIDAZOLES AS FOG INHIBITORS  
Brunello Mariani and Luigi Basaglia, Milan, Italy, assignors to Ferrania, S.p.A., Milan, Italy  
No Drawing. Filed Sept. 29, 1965, Ser. No. 491,390  
Int. Cl. G03c 1/34

U.S. Cl. 96—109

8 Claims

### ABSTRACT OF THE DISCLOSURE

Silver halide photographic emulsions are shown containing a 2-amino imidazole as a fog inhibitor.

This invention relates to the stabilization of photographic silver halide emulsions by 2-amino-benzimidazoles.

It is known that photographic emulsions coated onto a support have a tendency to lose desirable photographic characteristics upon aging. In particular, loss of sensitivity and the appearance of chemical fog is often observed. To minimize such changes various stabilizers have been added to the photosensitive emulsion. Such stabilizers include sulfonic or seleninic acids, triazoles, tetrazoles, indazoles, mercaptoazoles, diaryl-iodonium salts, potassium bromide, etc. Although certain benzimidazoles have been suggested for this purpose, in practice they tend to cause undesirable loss of sensitivity.

An object of this invention is to provide new photographic stabilizers and stabilized photosensitive layers.

Still another object is to provide a means for stabilizing photosensitive layers without objectionable loss of sensitivity due to the presence of stabilizers.

Other objects and advantages will become apparent from the following disclosure.

It has been found that efficient stabilization of photosensitive silver halide emulsions and fog inhibition can be achieved without a significant loss in sensitivity by incorporating in the emulsion a 2-amino imidazole, preferably having the structure



wherein D represents atoms necessary to complete an aromatic ring moiety, such as benzene or naphthalene.

## 2

These compounds may also exist in the imine form as



The aromatic moiety may be unsubstituted or substituted, for example with alkyl, aryl, aralkyl, alkoxy, halogen, nitro, sulfamide, etc. without affecting its utility as a stabilizer. Although the mechanism is not fully understood, it is believed that the ability of the compounds of this invention to exist in the form of either the imidazole or imine may be important in achieving stabilization without significant sensitivity loss.

The stabilizers of this invention are normally used in amounts from 5 to 100 milligrams per kilogram of wet photosensitive emulsion, to which they may be added in water, alcohol or acetone solution, preferably after the remelting or second digestion and prior to coating the support or film base. These stabilizers are particularly efficient when used in gelatin emulsions of silver halide, e.g. silver chloride, silver bromide-silver iodide, silver bromide-silver chloride. Their use does not preclude the use of conventional emulsion additives, including optical sensitizers, chemical sensitizers, gold, platinum, palladium, rhodium, iridium, tellurium and cadmium salts, color formers, surface active agents, hardeners, etc.

The following examples are presented for purposes of illustration and not for purposes of limitation.

Variable quantities of stabilizers of the above-mentioned type were added to 1 kilogram samples of the fast type gelatin emulsion containing silver bromide and silver iodide (10% silver halides of which 96% were bromide and 4% were iodide). The emulsions were then coated onto photographic film base. All samples were sensitometrically checked after coating without aging and after coating and accelerated aging (20 days at 50° C. and 40% relative humidity). Results are given in Table I.

In Table II the examples were prepared and tests in the same manner as the examples in Table I, the emulsion being further optically sensitized with N,N-diethyl-mesomethylthiobarboxyamine iodide.

As will be seen in the following tables, the sensitivity does not appear to be significantly altered by the presence of the stabilizers. Similar results were obtained when the stabilizers of Table I were incorporated into an emulsion of silver chloride-silver bromide of the type used for fast enlargement papers.

TABLE I

| Stabilizer                        | Mg per kg. of emulsion | Fresh |                      | Aged |                      |
|-----------------------------------|------------------------|-------|----------------------|------|----------------------|
|                                   |                        | Fog   | Relative sensitivity | Fog  | Relative sensitivity |
| Example:                          |                        |       |                      |      |                      |
| 1. None                           |                        | 0.05  | 100                  | 0.25 | 73                   |
| 2. 2-aminobenzimidazole           | 5                      | 0.04  | 100                  | 0.18 | 85                   |
| 3. do                             | 25                     | 0.04  | 100                  | 0.10 | 95                   |
| 4. do                             | 100                    | 0.04  | 100                  | 0.09 | 96                   |
| 5. 2-amino-naphthimidazole        | 5                      | 0.04  | 105                  | 0.10 | 97                   |
| 6. do                             | 25                     | 0.03  | 102                  | 0.09 | 99                   |
| 7. do                             | 100                    | 0.02  | 100                  | 0.08 | 99                   |
| 8. 2-amino-5-methoxybenzimidazole | 5                      | 0.04  | 104                  | 0.09 | 99                   |
| 9. do                             | 25                     | 0.03  | 100                  | 0.08 | 99                   |
| 10. do                            | 100                    | 0.03  | 100                  | 0.08 | 99                   |
| 11. 2-amino-5-nitrobenzimidazole  | 5                      | 0.03  | 100                  | 0.08 | 100                  |
| 12. do                            | 25                     | 0.02  | 95                   | 0.06 | 100                  |
| 13. do                            | 100                    | 0.02  | 90                   | 0.04 | 98                   |
| 14. 2-amino-5-chlorobenzimidazole | 5                      | 0.04  | 100                  | 0.09 | 98                   |
| 15. do                            | 25                     | 0.03  | 100                  | 0.06 | 98                   |

TABLE II

| Example: | Stabilizer                     | Mg per<br>kg. of<br>emulsion | Fresh |                         | Aged |                         |
|----------|--------------------------------|------------------------------|-------|-------------------------|------|-------------------------|
|          |                                |                              | Fog   | Relative<br>sensitivity | Fog  | Relative<br>sensitivity |
| 16.      | None                           | 0.06                         | 100   | 0.24                    | 81   |                         |
| 17.      | 2-amino-5-methoxybenzimidazole | 5 0.04                       | 100   | 0.06                    | 102  |                         |
| 18.      | do                             | 25 0.03                      | 100   | 0.06                    | 98   |                         |
| 19.      | do                             | 100 0.02                     | 99    | 0.04                    | 95   |                         |
| 20.      | 2-amino-naphthimidazole        | 5 0.05                       | 100   | 0.09                    | 108  |                         |
| 21.      | do                             | 25 0.03                      | 100   | 0.05                    | 100  |                         |
| 22.      | do                             | 100 0.02                     | 100   | 0.04                    | 96   |                         |
| 23.      | 2-amino-5-nitrobenzimidazole   | 5 0.04                       | 95    | 0.06                    | 98   |                         |
| 24.      | do                             | 25 0.02                      | 90    | 0.06                    | 95   |                         |

The embodiments of the invention in which an exclusive property or privilege is claimed are defined as follows:

1. A photosensitive silver halide emulsion layer containing therein as a fog inhibitor a stabilizing amount of a 2-amino imidazole of the formula



wherein D represents atoms necessary to complete an aromatic ring moiety.

2. A photosensitive silver halide emulsion layer containing therein a stabilizing amount of 2-aminobenzimidazole as a fog inhibitor.

3. A photosensitive silver halide emulsion layer containing therein a stabilizing amount of 2-amino naphthimidazole as a fog inhibitor.

4. A photosensitive silver halide emulsion layer containing therein a stabilizing amount of 2-amino-5-methoxybenzimidazole as a fog inhibitor.

5. A photosensitive silver halide emulsion layer containing therein a stabilizing amount of 2-amino-5-nitrobenzimidazole as a fog inhibitor.

6. A photosensitive silver halide emulsion layer containing therein a stabilizing amount of 2-amino-5-chlorobenzimidazole as a fog inhibitor.

7. An aqueous silver halide emulsion containing therein from 5 to 100 milligrams per kilogram of emulsion of a 2-amino imidazole of the formula



where D represents atoms necessary to complete an aromatic ring moiety.

8. An aqueous silver halide emulsion containing therein from 5 to 100 milligrams per kilogram of emulsion of 2-amino benzimidazole, 2-amino naphthimidazole, 2-amino-5-methoxy benzimidazole or 2-amino-5-chlorobenzimidazole.

#### References Cited

##### UNITED STATES PATENTS

- 2,324,123 7/1943 Weissberger ----- 96—109 X  
3,023,103 2/1962 Dersch et al. ----- 96—107 X  
3,255,202 6/1966 Johnson ----- 96—109 X

##### FOREIGN PATENTS

- 390,037 3/1933 Great Britain.

NORMAN G. TORCHIN, Primary Examiner

R. E. FICHTER, Assistant Examiner